

## UNITED STATES PATENT OFFICE

2,552,204

## PRODUCTION OF CAST IRON

Henton Morrogh, Alvechurch, Birmingham, England, assignor to The British Cast Iron Research Association, Alvechurch, Birmingham, England

No Drawing. Application October 25, 1949, Serial No. 123,537. In Great Britain October 30, 1948

11 Claims. (Cl. 75—130)

1

This invention relates to the production of cast iron, and more particularly to methods for the introduction of magnesium into cast iron.

Owing to its volatility and inflammability it is wasteful and dangerous to attempt to add magnesium metal to molten iron, and when it is desired to introduce magnesium into cast iron it has been proposed to alloy the magnesium first with a metal such as nickel so as to minimize the loss of magnesium and to limit the risk of fire.

We have found that under certain conditions magnesium may be introduced into cast iron by the use of a reducible magnesium compound such as magnesia or a compound convertible into magnesia by the action of heat; such compounds are for example magnesium carbonate, including magnesite, dolomite and chrom-magnesite, or organic magnesium salts such as magnesium oxalate. We have found that when molten iron at temperatures above 1650° C. is brought into contact with magnesia (or compounds generating magnesia at such temperatures) reduction of the oxide takes place and magnesium metal becomes available for the desulphurisation of the iron and, when the sulphur is or falls below 0.02 per cent, for solution in the iron.

It is known that silicon and ferrosilicon are able to reduce magnesium oxide at temperatures above 1100° C. to metallic magnesium. We have found that this reaction can be brought about by placing a mixture of magnesia (or magnesia-generating compounds) and silicon or ferrosilicon in contact with molten iron above 1100° C., and the magnesium produced is, as above, available for desulphurising and dissolving in the iron.

It is an object of the present invention to provide a method for introducing magnesium into cast iron. Another object is to provide a method for the desulphurisation of cast iron by means of magnesium. A further object is to provide a method for the production of grey cast iron in which the free carbon is present as graphite predominantly in the form of nodules. A still further object is to provide a method for the production of alloys of iron and magnesium. Other objects will appear from the following description.

These objects are achieved by the present invention according to which magnesium is introduced into cast iron by bringing the molten iron into contact with magnesia or a magnesia-generating compound at temperatures above 1650° C., or with a mixture of magnesia (or a magnesia-generating compound) and silicon or ferrosilicon at temperatures above 1100° C. If the iron originally contains more than 0.02 per cent by weight

2

of sulphur the excess sulphur is first removed by the magnesium, and unless desulphurisation is the sole aim, sufficient magnesia or magnesia mixture must be employed to deal with this sulphur and to enter into solution in the iron.

The reduction by silicon or ferrosilicon occurs more readily in the presence of small proportions of halides, such as magnesium chloride, calcium fluoride, or magnesium fluoride.

- 10 A convenient method of introducing the magnesium is to form a mixture of magnesia or burnt dolomite with a ferrosilicon containing, for example, 60–99% by weight of silicon, into briquettes with a suitable binding agent such as sodium silicate, bentonite or, preferably, Sorel cement. The briquetted bonded mixture may be plunged beneath the surface of the molten iron above 1100° C. in the ladle, and held there until sufficient magnesium has dissolved in the iron.
- 15 The briquettes should contain magnesia, lime and silicon (or the equivalent amount of ferrosilicon) in approximately the proportions indicated by the equation:
- 20



- 25 i. e. 80 parts by weight of magnesia, 112 parts of lime and 28 parts of silicon. Dolomite burnt at 950–1000° C. provides a mixture of magnesia and lime in the proportion 45:55, which is sufficiently near the stoichiometric proportion for the purpose. The ingredients are ground to pass at least 80 mesh and well mixed. If bentonite is to be used as binder, 5% of water is added to the finely powdered mixture and the whole is ground up with 5% of bentonite, briquetted and allowed to set, and finally dried at 200° C.

The addition of 5% of calcium fluoride to the finely powdered mixture improves its activity.

- 30 Alternatively, to the finely powdered mixture 40 may be added 5% of water and 5% of magnesium chloride, which acts both as a binder and an accelerator. A similar result may be obtained by treating the finely powdered mixture with up to 5% by weight of a 20% aqueous hydrochloric acid solution, whereby part of the oxides is converted into chlorides.

The invention thus provides a new and practicable method of introducing magnesium into molten iron by the use of magnesia or a magnesia-generating compound.

- 45 In the absence of elementary silicon temperatures above 1650° C. are necessary; but if the magnesia is associated with silicon, reduction to magnesium metal takes place at 1100° C. and 50 proceeds more readily at 1250° or higher. The

magnesia, with or without silicon, may be applied as a refractory lining to the walls of the furnace or the runs, or the ladle, always bearing in mind that unless the magnesia is associated with a due proportion of silicon temperatures above 1650° C. must be used. More conveniently the magnesia-silicon mixture is briquetted as described and held under the surface of the molten iron in the ladle, at temperatures of 1100° or higher, until sufficient has dissolved.

Magnesium is a well-known desulphurising agent, and the present invention provides a convenient method of reducing the sulphur content of iron during casting.

When magnesium has been used in quantity more than sufficient to reduce the sulphur content of the cast iron to below 0.02%, magnesium metal dissolves in the iron, and an alloy containing as much as 1% of magnesium can be produced in this way.

If the iron contains sufficient carbon, or additional carbon is provided, so that after casting a grey cast iron hypereutectic in respect of carbon results, the graphite in the cast iron will, when the magnesium added is more than sufficient to reduce the sulphur content to below 0.02 per cent, be predominantly in the nodular form and the cast iron will have the greatly improved properties described in my Patent No. 2,488,511. As in the process of that patent it is advantageous, after the introduction of the nodulising agent (in this case magnesium) to add a graphitising agent, e. g. ferrosilicon, calcium silicide, or graphite.

I claim:

1. A process for the introduction of magnesium metal into cast iron which comprises bringing the molten iron into contact with magnesia at temperatures at which reduction of the magnesia to magnesium takes place.

2. A process as claimed in claim 1 in which the magnesia is produced in situ by decomposition of a magnesia-generating compound.

3. A process for the introduction of magnesium metal into cast iron which comprises bringing the molten iron at temperatures above 1100° C. into contact with magnesia and silicon.

4. A process as claimed in claim 3 in which the magnesia is produced in situ by decomposition of a magnesia-generating compound.

5. A process for the introduction of magnesium metal into cast iron which comprises bringing the molten iron at temperatures above 1100° C. into contact with a briquette compounded from a magnesia-providing compound, selected from the group consisting of magnesia, magnesium carbonate, dolomite, chrome-magnesite and organic salts of magnesium, and a silicon-providing com-

pound selected from the group consisting of silicon and ferrosilicon, the briquette being held below the surface of the molten iron in the ladle until sufficient magnesium has dissolved.

6. A process as claimed in claim 5 in which the briquette contains, in addition to the magnesia-providing compound and the silicon-providing compound, an accelerator selected from the group consisting of calcium fluoride and magnesium chloride.

7. A process for the desulphurisation of cast iron which comprises bringing the molten iron at temperatures above 1100° C. into contact with magnesia and silicon, these ingredients being applied in such quantity as to provide enough magnesium metal to combine with the amount of sulphur to be removed.

8. A process for the production of a grey cast iron in which the free carbon content is at least predominantly in the form of nodular graphite which comprises treating a suitable molten iron at temperatures above 1100° C. with magnesia and silicon in such quantity as to provide more than sufficient magnesium metal to reduce the sulphur content of the iron to 0.02%, a suitable molten iron for this purpose being one which on casting yields a grey cast iron hypereutectic in relation to carbon.

9. A process as claimed in claim 8 which includes the further step of adding to the molten iron, after the introduction of the magnesium, a graphitising agent selected from the group consisting of ferrosilicon, calcium silicide and graphite.

10. A briquetted composition, suitable for the introduction of magnesium into cast iron, containing magnesia, calcium oxide and a silicon-providing substance, the magnesia and the silicon being present in substantially stoichiometric proportions, together with a magnesium chloride cement which acts as a binding and accelerating agent.

11. A briquetted composition as claimed in claim 10 in which said magnesium chloride cement is Sorel cement.

HENTON MORROGH.

#### REFERENCES CITED

The following references are of record in the file of this patent:

#### UNITED STATES PATENTS

| Number    | Name          | Date          |
|-----------|---------------|---------------|
| 1,119,643 | Saklatwalla   | Dec. 1, 1914  |
| 1,239,178 | Grosvenor     | Sept. 4, 1917 |
| 2,103,976 | Suchy et al.  | Dec. 28, 1937 |
| 2,282,241 | Peake         | May 5, 1942   |
| 2,485,760 | Millis et al. | Oct. 25, 1949 |